

March 16, 1937.

J. H. STRADLEY

2,074,031

CONTINUOUS DYEING PROCESS

Filed May 11, 1935



J.H.Stradley INVENTOR.

BY *John L. Seymour* ATTORNEY.

## UNITED STATES PATENT OFFICE

2,074,031

## CONTINUOUS DYEING PROCESS

James H. Stradley, Carneys Point, N. J., assignor  
to E. I. du Pont de Nemours & Company, Wil-  
mington, Del., a corporation of Delaware

Application May 11, 1935, Serial No. 21,017

2 Claims. (Cl. 8-5)

This invention relates to dyeing. More par-  
ticularly the invention relates to a continuous  
method of dyeing. The invention has particular  
application to the dyeing of materials such as  
5 yarn or fabric which are in considerable lengths,  
and will be described in relation to the dyeing of  
a roll of cotton cloth. It is to be understood,  
however, that this particular description does not  
limit the invention beyond the scope of the ap-  
10 pended claims.

There has been described in prior art a method  
which involves dyeing a roll of cotton cloth with an  
azo dyestuff containing a free amino group, diazo-  
15 tizing the dyestuff on the dyed cloth and coupling  
it to it, while still on the fiber, an azo dyestuff cou-  
pling component. In that process, the first dye-  
ing is carried out on a "jigger", the essentials of  
20 which include a tank, a roller at each side and  
one at the bottom of the tank. The cloth is wound  
on one roller, passed under the roller in the tank,  
and attached to the other roller; the tank is filled  
25 with dye solution, the cloth is drawn back and  
forth through the dye bath, the temperature is  
raised almost to boiling, and the material is  
given four to six additional passages through the  
30 solution. When the desired shade has been ob-  
tained the tank is drained, filled with cold water,  
and the material rinsed by repeated passages  
through the water.

35 The rinsing bath is drained off, the tank is filled  
with a diazotizing bath heated to 60-70° F., the  
cloth is twice passed through the bath, the ma-  
chine is drained and filled with fresh water, and  
the cloth is again rinsed. The tank is once more  
40 drained, is filled with a coupling bath containing  
an azo dyestuff coupling component, and the cloth  
is given two passages at 60-70° F. to form the  
final dye. The tank is emptied, filled with fresh  
water, the material is passed through until it is  
45 thoroughly rinsed, the rinse water is drained off,  
the tank is filled with a soap bath, and the cloth  
is soaped and rinsed in warm, and in cold water.  
This method requires from three to five hours  
for completion.

50 Where light shades are wanted, the original  
dyeing can be carried out in the above process by  
the so-called "padding" method, which differs  
from the jigger method only in that the first dye-  
ing of the undyed fiber is carried out by a single  
55 passage through the dyestuff solution.

Attempts have heretofore been made to dye by  
this method continuously: A number of tanks  
have been alined and the cloth has been passed  
through them in succession. Thus, in one meth-  
od the original dyestuff was applied by padding,

and the diazotization and development were ac-  
complished by passing the cloth through the  
alined tanks containing a concentrated diazotizing  
bath heated to 60-70° F., a rinsing bath, a  
concentrated developer bath, and as many rinses  
5 and soapings as was advantageous. The cloth  
was dried by passage over heated rollers.

The value of the method described in the pre-  
ceding paragraph was limited because it was  
necessary for the cloth to remain in contact with  
10 the diazotizing and developing agents for the  
period of time required for the slowest bath to  
operate, which in almost all cases proved exces-  
sive; because the use of very concentrated diazo-  
tizing and developing baths reduced the time of  
15 immersion but entailed an inability to properly  
"expose" the material; and because the varia-  
tion in the rate of development of different dyes,  
and in the shades obtained, limited the process  
to use with a very few dyestuffs.

Comparing the methods of the prior art, effec-  
tive diazotization was carried out in the inter-  
mittent method at low concentrations and low  
temperatures, temperatures above 80° F. being  
undesirable. A typical bath contained per 100  
20 gallons of water 1.5 pounds of sodium nitrite,  
2.5-3.0 pounds of sulfuric acid (66° Bé.) or  
1.87-2.25 pounds hydrochloric acid (20° Bé.), and  
the temperature would be held at 60-70° F. The  
25 diazotization bath of the continuous process of  
the prior art contained, per each 100 gallons of  
water, 12 pounds of sodium nitrite, 9.4 pounds  
of sulfuric acid (66° Bé.) or 21 pounds hydro-  
chloric acid (20° Bé.), and was held at a tem-  
30 perature of 60-70° F. The coupling bath of the  
35 intermittent prior art process contained (using  
beta naphthol in illustration), per 100 gallons of  
water, 0.5 pounds of betanaphthol, and 0.5 pounds  
of caustic soda at a temperature of 60-70° F. The  
continuous prior art process contained per 100  
40 gallons of water, 33.0 pounds of beta naphthol  
and 16.5 pounds of caustic soda.

It is an object of the invention to dye materials  
by a continuous method, which is equally ap-  
plicable to all dyestuffs substantive to cotton and  
45 regenerated cellulose and having a diazotizable  
amino group, which is much quicker than prior  
methods, which eliminates concentrated baths  
and long immersions, and which is both economi-  
cally and technically satisfactory.

The objects of the invention are attained,  
generally speaking, by passing cotton or regen-  
erated cellulose dyed with a dyestuff having a  
free amino group in single immersions sequenti-  
ally through diazotizing and coupling baths main- 55

tained at a temperature upward of 100° F. and preferably at about 140° F. The objects of the invention are in some degree attained by the details of the means and method more fully herein after described.

The process is illustrated in a preferred embodiment in the accompanying drawing, showing a diagrammatic representation of the dyeing of a roll of cloth, in which X is the roller holding the roll of cloth before applying the process; Y is the winding roller upon which the processed cloth may be collected; R are rollers, all, some, or none of which may be driven. In the preferred form of the invention the rollers outside the tanks will be driven and those within the tank will be freely mounted. Driers, not shown, may be located between tank G and roller Y.

On the roller X is wound dyed cloth of which the dyestuff has a free amino group. The tank A contains a diazotizing bath. In the preferred form of the invention that bath contains per 100 gallons of water 2½ to 3 pounds of sodium nitrite, 10 to 12½ pounds of sulfuric acid (66° Bé.) or 8½ to 10 pounds of hydrochloric acid (20° Bé.), and will be maintained at a temperature of 140° F. The tank B contains running cold water, but in some instances it can be replaced by a shower bath. The rollers R between tanks may, when it is advantageous, have complementary pressure rollers R' to squeeze excess moisture out of the cloth; the moisture so expelled may be caught in a trough T and conducted away from the process or back to the tank A. After the cold-water rinse in tank B, the cloth dyed with the diazotized dyestuff is drawn into tank C which contains a developing bath. The developer selected by the dyer will depend on the color and shade desired in the final dye. An exemplary bath contained 1½ to 2 pounds of beta naphthol, and 1½ to 2 pounds of caustic soda per 100 gallons of water, heated at about 140° F. The other azo dyestuff coupling components may be used in place of the beta naphthol. For instance, 1½ to 2 pounds of 1-phenyl-3-methyl-pyrazolone, or 1 to 1½ pounds of 2:4-diamino-toluene produce similar results when used with 1 to 1½ pounds of caustic soda. Other coupling components whose use is contemplated include: hydroxy aryls such as beta naphthol and resorcinol; amino aryls such as 2:4-diamino-toluene, 1:3-diamino-benzene, and ethyl-beta-naphthylamine; hydroxy aryl carboxylic acids such as beta-hydroxy-naphthoic acid and its amides; pyrazolones such as methyl-phenyl pyrazolone, amino-aryl-pyrazolone, and aryl-carboxy-pyrazolone; and aceto-acet arylids such as aceto-acet-anilide. Sulfonic acid derivatives of the above classes can be used, but in many cases they tend to solubilize the dye to an undesirable extent. This listing of coupling components is exemplary of classes not an exhaustive list of compounds.

Passing from tank C, the cloth with the newly-developed dyestuff is rinsed in cold water in tank D, soaped at 120-140° F. in box E which contains about three pounds of soap to each 100 gallons of water, rinsed in warm water (about 120° F.) in box F, and in cold water (preferably running) in box G. The dyed and washed cloth may, if desired, be dried before winding on roller Y.

The temperature of 140° F. is not an operative upper limit, satisfactory results being obtainable upwardly thereof, but it is a temperature at which

excellent efficiency is obtained and above which the evolution of gases is excessive.

An advantage of the invention is a continuous process of dyeing useful with substantially all dyestuff substantive to cotton and regenerated cellulose and capable of diazotization and development on the fiber. This advantage is illustrated by reference to the following colors, identified by the Color Index Number, which could not be successfully used by the old continuous process, but produce entirely satisfactory results when applied by my process.

CI-297 Diazotized and developed with beta naphthol  
 CI-317 Diazotized and developed with beta naphthol  
 CI-322 Diazotized and developed with beta naphthol  
 CI-323 Diazotized and developed with 2:4-diamino-toluene  
 CI-324 Diazotized and developed with 1-phenyl-3-methyl-pyrazolone  
 CI-324a Diazotized and developed with beta naphthol  
 CI-339 Diazotized and developed with beta naphthol  
 CI-401 Diazotized and developed with 2:4-diamino-toluene  
 CI-552 Diazotized and developed with 2:4-diamino-toluene  
 CI-625 Diazotized and developed with beta-naphthol  
 CI-812 Diazotized and developed with beta-naphthol

Another advantage of the invention is in the saving of time and labor in dyeing. In the jigger method three to five hours were required to complete the dyeing process. The continuous process of the prior art, when used with those few colors which could be successfully applied, acted in about three minutes per bath. My invention operates on cotton or regenerated cellulose with any dyestuff of the class described and reduces the time to about ten seconds per bath. Another advantage of my process is that the concentration of diazotizing and developing baths is about equal to the prior intermittent process and far lower than those of prior continuous processes.

The use of alkaline coupling baths in the examples is not a limitation to baths of that type. The coupling bath will be made alkaline, neutral, or acid in accordance with the dictates of good practice relating to each particular coupling component.

The fastness to washing, and discharge properties of the dyestuffs when produced by my new continuous method are equal to those of the old prolonged jigger process.

As many apparently widely different embodiments of this invention may be made without departing from the spirit and scope thereof, it is to be understood that I do not limit myself to the specific embodiments thereof except as defined in the appended claims.

I claim:

1. A continuous method of dyeing which comprises passing a material of the class consisting of cellulose and regenerated cellulose dyed with an azo dyestuff substantive to cotton or regenerated cellulose having a diazotizable amino group through a diazotizing bath heated to about 140° F. and a coupling bath containing an azo dyestuff coupling component, the material being

5

10

20

25

35

40

45

50

55

60

65

70

75

immersed in said diazotization bath for a period of time not greater than about ten seconds.

2. A continuous method of dyeing which comprises passing a material of the class consisting of cellulose and regenerated cellulose dyed with an azo dyestuff substantive to cotton or regenerated cellulose and having a diazotizable amino group, through a diazotizing bath heated to about 140° F., and a coupling bath containing an azo dyestuff coupling component selected from the group consisting of beta naphthol, 2:4-diaminotoluene and 1-phenyl-3-methyl-pyrazolone, the material being immersed in said diazotization bath for a period of time not greater than about ten seconds.

JAMES H. STRADLEY.